

# United States Patent [19]

Mimino et al.

[11] 3,847,600

[45] Nov. 12, 1974

[54] HIGH TEMPERATURE ALLOY STEEL

[75] Inventors: **Tohru Mimino; Kazuhisa Kinoshita; Keisuke Hattori**, all of Kawasaki, Japan

[73] Assignee: **Nippon Kokan Kabushiki Kaisha**, Kawasaki-shi, Kanagawa-ken, Japan

[22] Filed: May 9, 1973

[21] Appl. No.: 358,797

**Related U.S. Application Data**

[63] Continuation of Ser. No. 63,623, Aug. 13, 1970, abandoned.

[30] **Foreign Application Priority Data**

Aug. 8, 1969 Japan..... 44-67174

[52] U.S. Cl..... 75/126 C, 75/126 E, 75/126 F, 75/126 J, 75/126 P

[51] Int. Cl..... C22c 39/14, C22c 39/26

[58] **Field of Search**..... 75/126 C, 126 F, 126 E, 75/126 J, 126 P

[56]

**References Cited**

UNITED STATES PATENTS

|           |         |               |          |
|-----------|---------|---------------|----------|
| 3,539,338 | 11/1970 | Mimino.....   | 75/126 C |
| 2,109,118 | 2/1938  | Naumann ..... | 75/126 F |
| 3,044,872 | 7/1962  | Hayes.....    | 75/126 C |
| 2,572,191 | 10/1951 | Payson .....  | 75/126 F |
| 3,290,183 | 12/1966 | Ohtake.....   | 75/126 C |
| 3,201,232 | 8/1965  | Thier .....   | 75/126 C |

*Primary Examiner*—L. Dewayne Rutledge

*Assistant Examiner*—Arthur J. Steiner

*Attorney, Agent, or Firm*—Flynn & Frishauf

[57]

**ABSTRACT**

An alloy steel suitable for use at high temperatures, having excellent corrosion resistance, creep strength, hot forming characteristics and weldability. The steel is an inexpensive ferrite steel having a composition comprising C up to 0.10 percent, Si up to 1%, MN 0.3 – 1.20 percent, Cr 7-10 percent, Mo 0.3-1.5 percent V 0.1 – 0.3 percent, Nb 0.15 – 0.50 percent, B up to 0.012 percent, N up to 0.050 percent balance fe and incidental impurities.

**6 Claims, No Drawings**

## HIGH TEMPERATURE ALLOY STEEL

This is a continuation of application Ser. No. 63,623 filed Aug. 13, 1970, now abandoned.

U.S. Pat. No. 3,539,338 issued Nov. 10, 1970 discloses related subject matter.

This invention relates to a high temperature alloy steel, the alloy steel being an inexpensive ferrite high temperature steel having high creep rupture strength at temperatures up to about 650°C and having superior weldability.

There is a great demand for a high temperature alloy steel tube having high temperature strength and high temperature corrosion resistance at low cost for use in operations under conditions of high temperature and high pressure such as in steam-power units, petroleum refining processes and other petroleum industries.

Heretofore, several kinds of steel tubes have been used according to the conditions of temperature, pressure and atmosphere, but there has been proposed no steel tube of suitable characteristics for a temperature ranging from 550°C to 650°C. The ferrite steel groups of either 2.25% Cr—1% Mo steel, 5% Cr—0.5% Mo steel or 9% Cr—1% Mo steel and the austenite stainless steel groups of either 18% Cr—8% Ni or 18% Cr—Ni—Ti have been conveniently applied under the above high temperature condition. However, 2.25% Cr—1% Mo ferrite steel does not have a sufficiently high temperature corrosion resistance to be used at a temperature of over about 575°C and both the 5% Cr 0.5% Mo and 9% Cr—1% Mo ferrite steels are so low in creep rupture strength and so high in quenched hardness in the heat affected portions of a welded structure as to result in cracks. Austenitic stainless steel is very expensive because of the large quantity of expensive Ni addition.

The present invention has been developed on the

cent provides a high temperature corrosion resistance up to 650°C similar to that of 9% Cr—1% Mo ferrite alloy steel, and Mo addition of 0.3 to 1.5% Nb addition of 0.15 to 0.50% and V addition of 0.1 to 0.3% form stable carbide and nitride at high temperature to improve high temperature strength. This high temperature strength may be further improved by either individual or combined addition of 0.001—0.012 percent boron and 0.015—0.050 percent nitrogen in addition to the above listed alloying compositions.

Preferred high temperature alloy steel of the present invention consists essentially of the following elements in the following weight percentages:

|    |            |              |
|----|------------|--------------|
| 15 | carbon     | 0.04—0.06%   |
|    | silicon    | 0.45—0.60%   |
|    | manganese  | 0.50—0.75%   |
|    | chromium   | 7.75—8.50%   |
|    | molybdenum | 0.9—1.00%    |
|    | vanadium   | 0.15—0.25%   |
|    | niobium    | 0.30—0.35%   |
|    | boron      | 0.007—0.008% |
|    | nitrogen   | 0.011—0.030% |

the balance being iron and incidental impurities.

The high temperature alloy steel of the present invention is characterized in that the maximum hardness of weld heat affected portions is so low that there is little possibility for low temperature cracking while welding. This excellent characteristic is due to the fact that C content is limited to less than 0.10 percent and is stabilized because of the combination of carbon into such carbides as NbC, VC and the like.

The embodiments of the present invention will be described in detail hereinafter.

The typical chemical compositions of this invention alloy steel is shown in the following Table 1.

Table 1

| Marks | C    | Si   | Mn   | Cr   | Mo   | V    | Nb   | N     | B     |
|-------|------|------|------|------|------|------|------|-------|-------|
| A     | 0.06 | 0.53 | 0.73 | 8.51 | 0.98 | 0.21 | 0.32 | 0.011 | —     |
| B     | 0.05 | 0.48 | 0.65 | 8.32 | 0.97 | 0.22 | 0.35 | 0.014 | 0.008 |
| C     | 0.05 | 0.61 | 0.68 | 7.76 | 0.91 | 0.21 | 0.35 | 0.027 | —     |
| D     | 0.04 | 0.46 | 0.56 | 7.88 | 0.92 | 0.17 | 0.35 | 0.025 | 0.007 |

basis of a careful study and numerous experiments with the afore-mentioned facts, namely the necessity for a high temperature alloy steel manufactured at low cost for use in modern industries and the defects of the conventionally used ferrite steels, in order to provide a ferritic heat resistant alloy steel of excellent mechanical properties at low cost. In other words, this invention has made an improvement in high temperature strength, hot forming properties, cold forming properties and weldability of a 9% Cr—1% Mo ferrite alloy steel.

The high temperature alloy steel of this invention comprises less than 0.10% carbon, less than 1.0% silicon, 0.30—1.20% manganese, 7—10% chromium 0.3—1.5% molybdenum, 0.1—0.3% vanadium, 0.15—0.50% niobium and the balance being iron and incidental impurities.

The compositions of the present alloy steel will be described in detail as follows: Cr addition of 7 to 10 per-

cent provides a high temperature corrosion resistance up to 650°C similar to that of 9% Cr—1% Mo ferrite alloy steel, and Mo addition of 0.3 to 1.5% Nb addition of 0.15 to 0.50% and V addition of 0.1 to 0.3% form stable carbide and nitride at high temperature to improve high temperature strength. This high temperature strength may be further improved by either individual or combined addition of 0.001—0.012 percent boron and 0.015—0.050 percent nitrogen in addition to the above listed alloying compositions.

Preferred high temperature alloy steel of the present invention consists essentially of the following elements in the following weight percentages:

Table 2

| Kinds of Steel | Creep Rupture Strength (kg/mm <sup>2</sup> ) |                               |                               |                               |
|----------------|----------------------------------------------|-------------------------------|-------------------------------|-------------------------------|
|                | 600°C<br>10 <sup>3</sup> hrs.                | 600°C<br>10 <sup>4</sup> hrs. | 650°C<br>10 <sup>3</sup> hrs. | 650°C<br>10 <sup>4</sup> hrs. |
| 2.25% Cr—1% Mo | 1.01                                         | 7.3                           | 6.3                           | 4.0                           |
| 5% Cr—0.5% Mo  | 7.3                                          | 5.5                           | 4.5                           | 2.8                           |
| 9% Cr—1% Mo    | 8.0                                          | 6.0                           | 4.8                           | 3.2                           |
| This Invention | A                                            | 14.1                          | 11.5                          | 9.3                           |
| Alloy Steel    | B                                            | 14.1                          | 11.6                          | 9.5                           |
|                | C                                            | 15.0                          | 11.7                          | 9.5                           |
|                | D                                            | 15.0                          | 12.1                          | 10.0                          |
|                |                                              |                               |                               | 7.1                           |

As is seen from the above Table 2, the present invention alloy steels have as much as 1.5 times higher creep rupture strength than that of the 2.25% Cr—1% Mo steel having the highest creep strength among prior ferrite steels, and approximately twice as high creep rupture strength as those of 5% Cr—0.5% Mo steel and 9% Cr—1% Mo steel.

The next Table 3 shows the maximum strength of the weld heat affected portions of those alloy steels listed in Table 2.

Table 3

| Kinds of Steel       | Maximum Hardness of Weld Heat Affected Portions |     |
|----------------------|-------------------------------------------------|-----|
|                      | Maximum Hardness (HV)                           |     |
| 2.25% Cr—1% Mo steel | 340                                             | 360 |
| 5% Cr—0.5% Mo steel  | 410                                             | 430 |
| 9% Cr—1% Mo steel    | 440                                             | 460 |
| This Invention       | A                                               | 310 |
| Alloy Steel          | B                                               | 280 |
|                      | C                                               | 290 |
|                      | D                                               | 280 |

It is apparent from the above Table 3 that the maximum hardness of the alloy steels of this invention ranges from HV 280 to 310, being remarkably lower than the maximum hardness of the conventional alloy steels. It is concluded, therefore, that there is little possibility for low temperature cracking in the steels according to the present invention because of martensite transformation during the welding operation.

The alloy steel of the present invention is useful in fields requiring operation at temperatures up to 650°C and particularly for boilers, petroleum refining processes, general chemical industries, heat exchanger tubes of atomic furnaces and pipe line materials. As has been discussed hereinabove, this invention provides a high temperature alloy steel for the relatively inexpen-

sive ferrite group having high creep rupture strength up to temperatures of about 650°C being characterized in that the maximum hardness of weld heat affected portions is low and therefore low temperature cracks are unlikely to be caused while welding, thereby proving of great advantage in modern industries.

The embodiments of the invention in which an exclusive property or privilege is claimed are defined as follows:

10 1. A high temperature alloy steel having high creep rupture strength up to temperatures of about 650° consisting essentially of the following elements in the following weight percentages:

|            |                 |
|------------|-----------------|
| carbon     | less than 0.10% |
| silicon    | less than 1.0%  |
| manganese  | 0.30—1.20%      |
| chromium   | 7—10%           |
| molybdenum | 0.3—1.5%        |
| vanadium   | 0.1—0.3%        |
| niobium    | 0.15—0.50%      |
| boron      | up to 0.012%    |
| nitrogen   | up to 0.05%     |

15 25 the balance being iron and incidental impurities.

2. A high temperature alloy steel according to claim 1, containing 0.001 to 0.012 percent of boron.

3. A high temperature alloy steel according to claim 1, containing 0.015 to 0.050 percent of nitrogen.

30 4. A high temperature alloy steel according to claim 1, containing 0.001 to 0.012 percent of boron and 0.015 to 0.050 percent of nitrogen.

35 5. A high temperature alloy steel consisting essentially of the following elements in the following weight percentages:

|            |              |
|------------|--------------|
| carbon     | 0.04—0.06%   |
| silicon    | 0.45—0.60%   |
| manganese  | 0.50—0.75%   |
| chromium   | 7.75—8.50%   |
| molybdenum | 0.9—1.00%    |
| vanadium   | 0.15—0.25%   |
| niobium    | 0.30—0.35%   |
| boron      | 0.007—0.008% |
| nitrogen   | 0.011—0.030% |

40 the balance being iron and incidental impurities.

6. A high temperature alloy steel tube having high creep rupture strength up to temperatures of about 650° consisting essentially of the alloy steel of claim 5.

\* \* \* \* \*

UNITED STATES PATENT OFFICE  
CERTIFICATE OF CORRECTION

Patent No. 3,847,600 Dated November 12, 1974

Inventor(s) TOHRU MIMINO et al

It is certified that error appears in the above-identified patent and that said Letters Patent are hereby corrected as shown below:

On the first page, lefthand Column, [30]:

The priority date "Aug. 8, 1969" should be  
--Aug. 27, 1969--.

Signed and Sealed this  
*thirtieth Day of September 1975*

[SEAL]

*Attest:*

**RUTH C. MASON**  
*Attesting Officer*

**C. MARSHALL DANN**  
*Commissioner of Patents and Trademarks*